

June 4, 1935.

J. O'NEILL

2,003,695

WOVEN WIRE FABRIC

Filed Aug. 6, 1932



*Joseph O'Neill* INVENTOR

## UNITED STATES PATENT OFFICE

2,003,695

## WOVEN WIRE FABRIC

Joseph O'Neill, Port Chester, N. Y.

Application August 6, 1932, Serial No. 627,785

7 Claims. (Cl. 139—425)

This invention relates to improvements in woven wire fabrics such as are used on Fourdrinier and cylinder paper making machines and one of its objects is to provide a fabric or cloth 5 of longer wearing quality than heretofore available without altering in any way the drainage or other requirements for paper making purposes.

Another object of the invention is to provide a Fourdrinier wire cloth having greater durability 10 and strength without impairing its bending and flexing qualities, and of a relatively rustless, non-corrosive and non-electrolytic character.

Another object of this invention is to utilize in 15 a woven wire fabric wires composed of metal relatively soft with respect to steel and of tensile strength upwards of that of the usual bronzes and approaching that of steel.

Another object of this invention is to provide 20 a woven wire fabric which retains its relative flexibility and does not become over-brittle in use by reason of work-hardening or fatigue or crystallization or the like.

Another object of this invention is to provide 25 a woven wire fabric having special wires which do not cut or shear the remaining wires of the fabric.

Other objects will be apparent from the specification.

I have discovered that a Fourdrinier wire fabric 30 has a longer life and produces greater tonnage of paper when certain of its warp wires interposed at intervals across the entire width of the warp are made of a composition of copper, manganese and silicon, a mixture which may be termed a manganese-silicon-bronze.

Fourdrinier "wires" as generally made at the present time consist of interwoven wires of brass or phosphor bronze, of tensile strength substantially less than that of steel, which, although relatively pliant or flexible and resistant to corrosion and electrolysis, last for only a short period of time. Fabric composed of these coppery metals 40 readily wears down and loses resiliency which accelerates its destruction.

My improved fabric retains the pliancy or flexibility of such compositions of brass or phosphor bronze fabric to withstand the repeated and rapid bending and unbending of the fabric on the paper machine and is of equal or greater resistance to 45 corrosion and electrolysis and in addition increases both resistance to wear and tensile strength thereby increasing the life of the fabric. This is accomplished by increasing the durability and strength of the warp or longitudinal wires 50 upon which the major burden of wear and strain

falls, by substituting for some of the usual brass or phosphor bronze warp wires, strengthening warp wires of coppery metal essentially non-work-hardening and of higher tensile strength.

Such strengthening warp wires being of greater tensile strength than the remaining usual brass or phosphor bronze warp wires, lessen the longitudinal strain by reducing stretching of the fabric thereby keeping it resilient and elastic and increasing its wearing life; and being still of soft metal, do not cut the remaining wires in contact therewith; and being non-work-hardening, do not become brittle and fracture themselves prematurely.

In a plain woven fabric, I have found that such strengthening wires consisting of approximately 96% copper, 1% manganese and 3% silicon preferably soft-annealed and used as every sixth warp wire and the remaining warp wires of the usual brass or phosphor bronze and the shuttle wires of brass, gives successful results by way of increased life of the fabric and increased tonnage of paper. These strengthening wires may be of the same size and spacing as the remaining warp wires so as not to project above the surface and 20 may conform in all other respects to standard practise for the construction and operation of Fourdrinier wire fabrics as to drainage, mesh and other characteristics.

The accompanying drawing is a view greatly 30 enlarged and not to scale of part of a Fourdrinier "wire" embodying my invention.

The fabric when made according to my invention may comprise the usual brass shuttle or transverse wires *a*, groups *1*, *2* and *3* of a desired 35 number of the usual brass or phosphor bronze longitudinal or warp wires *b*, and warp wires *c*, of tough coppery alloy such as approximately 96% copper, 1% manganese and 3% silicon drawn and annealed and interposed at regular intervals 40 across the entire width of the warp. In the drawing, the weave shown is plain or standard, and all wires *a*, *b*, and *c* are shown of the same size and equally spaced apart but my improvement is intended to cover variations in size and spacing of the wires and any type of weave such as twilled weave, or reinforced weave as shown 45 in my U. S. Patent Number 1,593,668 patented July 27, 1926, or other type.

In the drawing, I have shown the groups *1*, *2* 50 and *3* of warp wires *b* as containing four wires each, which has been found suitable for the average Fourdrinier fabric but this is solely for illustrating purposes, as any desired number of wires *b* may be used in each group *1*, *2* and *3* and the 55

special strengthening wires *c* of copper alloy may be interposed between them. Sometimes it is desirable to strengthen the edges of the wire fabric and the strengthening wires *c* may then 5 adjoin each other or be in some other close arrangement to make the edges stronger.

While I have shown the special wires *c* of a preferred composition, other manganese-silicon bronzes may be used. The mixture may in some 10 cases range from about 82 to 96.5% copper, from about 3 to 15% silicon and from about 0.5 to 3.0% manganese. The tensile strength of the mixture may be upwards of 50000 pounds per square inch and may approach or equal that of steel. This 15 manganese-silicon bronze may be prepared in a manner known to those skilled in the art of mixing, drawing, and annealing bronzes.

Other bronzes may be employed such as mixtures of copper with small quantities of manganese or silicon or other bronzes or metals relatively soft with respect to steel and that have a tensile strength approaching that of steel or upwards of about 50000 pounds per square inch in 20 ultimate tensile strength.

25 And while I have shown my special wires as composing part only of the warp, they may be employed in whole or in part of the warp or shute.

I am aware of Fourdrinier wire fabrics made 30 by substituting some of the usual brass or phosphor bronze warp wires with warp wires of hard, non-coppery metal wires, but my invention is an improvement thereover. The bending and unbending of the fabric as it passes around the 35 rolls of the paper machine rapidly work-hardens and makes more brittle such hard metal wires causing them to break prematurely and also break or tear sections of the fabric thereby making it unfit for further use. The great difference between the physical properties of such hard metal 40 wires and the remaining brass or phosphor bronze wires subjects the latter in a Fourdrinier fabric to forces that cause shearing or tearing of the brass shute wires. Such hard metals being non-coppery metals are more subject to electrolytic 45 action when associated with brass or phosphor bronze in certain alkaline, salt or acid solutions which may be present in the manufacture of paper.

50 My invention, however, overcomes these difficulties. The relatively soft metal coppery alloy wires do not harden perceptibly in use and premature cracking of such wires themselves or of the fabric is thereby avoided. My special wires 55 work in harmony with the remaining wires in the fabric, neither reacting unfavorably upon the other to cut, shear, tear, weaken or otherwise be adversely affected mechanically, chemically, electrolytically or otherwise. My special strengthening wires of relatively soft metal retain their 60 high tensile strength, flexibility, and resiliency when used with the remaining wires with which they cooperate to resist frictional wear and give longer life to the fabric than heretofore available.

Also I am aware of fabrics of the prior art which I have used and which consisted of warp wires, some of brass and others of phosphor bronze, but my invention is an improvement thereover since among other reasons, these wires lacked the tensile strength of my present invention and did not have the long life wearing qualities of my improved fabric.

5 I have illustrated my invention as embodied in a wire fabric for use in a Fourdrinier paper making machine but as the invention is also useful in cylinder paper making and pulp treating machines, woven wire belts as conveyor belts, and for straining and bolting purposes or wherever it is desired to strengthen a member subjected 10 to force, I intend no limitations other than those imposed in the appended claims and such modifications as may occur to a person skilled in the art are intended to be included within the scope 15 of the claims.

20 What I claim is:

1. Paper-making and paper pulp treating woven wire fabric having warp wires of an alloy including copper, manganese and silicon.

2. Paper-making woven wire fabric as Fourdrinier or cylinder wire fabric having warp wires of an alloy including copper, manganese and silicon, at least some of said wires being disposed 25 in the central part of said fabric.

3. Fourdrinier paper-making woven wire fabric 30 having warp wires of an alloy including copper, manganese and silicon, some of said warp wires being disposed in the central portion of said fabric and others of said warp wires being disposed adjacent the two edges of said fabric.

35 4. Fourdrinier paper-making wire fabric having warp wires of an alloy including copper, manganese and silicon, said warp wires being disposed at the two edges of the fabric whereby 40 said edges are strengthened.

5. Fourdrinier woven wire fabric comprising interwoven warp and shute wires, said shute wires and some of said warp wires being of metal including copper and others of said warp wires consisting of an alloy including copper, manganese 45 and silicon interspersed among said first-mentioned warp wires at substantially regular intervals such as every fifth or sixth warp wire across substantially the entire width of the fabric warp.

6. Fourdrinier woven wire fabric comprising 50 interwoven warp and shute wires, said shute wires and some of said warp wires being of coppery metal such as the usual brass or phosphor bronze and others of said warp wires consisting of an alloy including copper, manganese and silicon 55 interspersed among said coppery metal warp wires at intervals across substantially the entire width of the fabric.

7. Fourdrinier paper-making wire fabric comprising interwoven warp wires and shute wires, 60 all of the warp wires of said fabric being of an alloy including copper, manganese and silicon.

JOSEPH O'NEILL.